

No. 895,163.

PATENTED AUG. 4, 1908.

S. O. COWPER-COLES.  
ELECTRODEPOSITION OF COPPER.

APPLICATION FILED MAY 20, 1907.

2 SHEETS—SHEET 1.

Fig. 1.



Witnesses.

J. K. Moore  
H. E. Bopp

Inventor.

Sherard O. Cowper-Coles  
Inventor  
by  
John L. Coles, atty.

No. 895,163.

PATENTED AUG. 4, 1908.

S. O. COWPER-COLES.  
ELECTRODEPOSITION OF COPPER.  
APPLICATION FILED MAY 20, 1907.

2 SHEETS—SHEET 2.

Fig. 2.



Witnesses.

J. K. Moore  
John E. Popp

Inventor.

Edward O. Cowper-Coles.  
Whitaker & Bowes <sup>37</sup> Atty.

# UNITED STATES PATENT OFFICE

SHERARD OSBORN COWPER-COLES, OF LONDON, ENGLAND.

## ELECTRODEPOSITION OF COPPER.

No. 895,163.

Specification of Letters Patent.

Patented Aug. 4, 1908.

Application filed May 20, 1907. Serial No. 374,805.

*To all whom it may concern:*

Be it known that I, SHERARD OSBORN COWPER-COLES, a subject of the King of Great Britain, residing at Grosvenor Mansions, 82 Victoria street, Westminster, London, England, have invented new and useful improvements in the Electrodeposition of Copper; and I do hereby declare that the following is a full, clear, and exact description of the invention, which will enable others skilled in the art to which it appertains to make and use the same.

My invention relates to an improved process for the electrodeposition of copper. Copper produced by the usual method of electrodeposition upon a stationary or slowly revolving cathode is found in practice to lack tensile strength and to be of a porous nature; attempts have been made to overcome this difficulty by rotating the cathode at a high speed or by burnishing the metal during electrodeposition but the burnishing is found to produce laminations. Now, I have found in practice that copper possessing the advantages of hard rolled copper of high tensile strength and free from porosity can be electrodeposited at a rapid rate by revolving the cathode at a peripheral speed of from 1,500 to 2,000 feet per minute when employing a current density of 200 amperes per square foot of cathode surface and an electrolyte containing 12.5 per cent. of copper sulfate and 13 per cent. of sulfuric acid at a temperature of 40° centigrade. I have also found that the tensile strength of the copper produced increases with the increase of the speed of revolution of the cathode above 1,500 feet per minute.

In order that my invention may be more clearly understood, I have illustrated in the accompanying drawings, one form of apparatus for carrying out my process, similar reference letters in which indicate identical parts throughout.

In the drawings, Figure 1 is a sectional ele-

vation of a suitable form of apparatus for carrying out the invention, and Fig. 2 is a plan view thereof.

*a* represents the electrolytic vat having an inlet *b* and an overflow outlet *c* for the electrolyte.

*d* is the cathode which is secured to the upper end of the spindle *e* mounted in bearings in the vat *a* and adapted to be rotated at the requisite speed through the medium of the bevel gear *e'*.

*f, f'* are the anode segments which are supported by means of the rods *f', f'* on the annular frame *g*. These anode segments are adapted to be adjusted in position relatively with the cathode *d* as the operation proceeds by means of the wedge-shaped projections *h, h* formed upon the said segments and which wedge-shaped projections engage with wedges *i, i* upon rods *j* vertically mounted within the vat *a* and provided at their upper projecting ends with screw threads *k*. Nuts *l* engage with the screw threaded portions *k* of these rods *j*, the said nuts bearing upon the supporting brackets *m* of the rods. By turning these nuts *k* the rods *j* can be raised so as to shift the anode segments *e* inwards to the desired extent.

Having now fully described and ascertained my said invention and the manner in which it is to be performed, I declare that what I claim is:

The process of electrodeposition of copper, which consists in passing a current of electricity of a density of 200 amperes per square foot of cathode surface from an anode to a cathode and revolving said cathode at a speed of 1500 or more revolutions per minute in an electrolyte consisting of approximately 12.5% of copper sulfate and 13% of sulfuric acid, substantially as described.

SHERARD OSBORN COWPER-COLES.

Witnesses:

JOHN E. BOUSFIELD,

C. G. REDFERN.